

## UNITED STATES PATENT OFFICE

FRANK O. WOODRUFF, OF QUINCY, MASSACHUSETTS, ASSIGNOR TO BECKWITH MANUFACTURING COMPANY, OF BOSTON, MASSACHUSETTS, A CORPORATION OF MASSACHUSETTS

## SHOE STIFFENER MATERIAL AND ART OF MAKING

No Drawing. Application filed January 18, 1930. Serial No. 421,814.

This invention relates to the production of sheet material intended more particularly for use in making shoe stiffeners such as counters or box toes. Such sheet material usually comprises a fibrous base, such as felt, saturated with an agent which under suitable treatment quickly becomes plastic or gelatinous but which quickly sets or hardens under atmospheric temperature conditions. 10 The sheet material is cut into stiffener blanks, which when subjected to treatment designed to plasticize or gelatinize the agent present therein becomes soft and limp, in which condition the blanks are moulded or shaped to 15 the desired form and permitted to set in such form. Various classes of agents may be used to impart the desired stiffness or rigidity to the moulded article, but cellulose derivatives such as the nitrate and acetate have 20 sometimes been preferred, not only because of the rapidity with which they undergo gelatinization when treated with suitable solvents, but also because they set rapidly under room 25 temperature conditions as the solvent is evaporated to produce a product characterized by its stiffness, resiliency, and permanency against varying atmospheric temperature conditions. An object of the present invention is to provide a shoe stiffener material in which a cellulose derivative capable of being gelatinized by a volatile solvent is uniformly distributed in such condition as to make possible a rapid, uniform, and substantially complete gelatinization by the solvent. In accordance with 30 the present invention, this object is attained by coating suitable papermaking fibrous material with a solution of the cellulose derivative, then beating the coated fibrous material to a pulpois condition suitable for forming into paper, and forming the beaten stock into a waterlaid felt on a paper machine. After 35 the coating of the fibrous material and before introducing it into the beater engine, the solvent of the cellulose derivative may be evaporated and recovered, in which case the derivative is deposited on and adheres to the fibers in a set condition and commingling of the solvent with the water used in the 40 beater engine in preparing the pulp is avoided. The fibrous material to be coated with the solution of the derivative may be in a loose, unwoven condition so that it may be admixed with the solution, or it may be in the form of a woven or knitted fabric so 45 that it may be impregnated or coated on one or both faces with the solution. A straight solution of only the derivative may be employed, but, if desired, agents less expensive than the derivative, such as rosin, may be 50 added in suitable proportion to the solution to increase the amount of solid material deposited upon the fibrous material upon removal of the solvent, but without materially interfering with the capacity of the derivative 55 for undergoing gelatinization by the action of a solvent. When nitrocellulose is the derivative, it may be compounded with camphor as celluloid. When the fibrous material, more or less coated with cellulose derivative, is beaten and run out into a waterlaid sheet on suitable papermaking machinery, e. g., a wet machine, and then dried, it is 60 found that the product is of high porosity and is not unlike ordinary paper in its flexibility, feel, and other characteristics. Such sheet material lends itself with especial facility to the operations of cutting into shoe 65 stiffener blanks and to skiving of the blanks at their marginal portions. The blanks may 70 be rapidly and uniformly impregnated with a solvent for the derivative, as by dipping thereinto, to effect a rapid and complete gelatinization of the cellulose derivative present 75 therein. A blank thus treated becomes sufficiently soft or limp to be easily formed or moulded to the shape of the last used in making the shoe, and upon the evaporation of the solvent becomes set in a stiff and resilient condition, in which condition it is practically 80 unaffected even by extreme atmospheric temperature conditions. One of the major advantages of a process such as described is that practically all the cellulose derivative used as a raw material 85 appears in the finished waterlaid sheet of fibers. Evidently the cellulose derivative initially deposited on and adherent to the fiber remains fixed to the fibers throughout beating and papermaking operations, as evi- 90 95 100

denced by the fact that there is little, if any, turbidity in the water removed from the paper machine during the paperforming operation, to indicate the presence of cellulose derivative therein. A substantial loss of the cellulose derivative used as a raw material is especially serious because of the comparatively high cost of such material. I lay stress on the economic phases of my process, because 5

10 I am aware that many years ago it was proposed to incorporate powdered celluloid into paper pulp in the beater engine, and then to run out the stock on a paper machine. Such a process, however, is commercially unfeasible, not only because of the expense incident to the step of pulverization, but more particularly because of the material loss of celluloid in the white water removed during formation of the paper.

15 Another important advantage possessed by my process is that it makes possible the use of celluloid-coated fabric clippings or other waste fibrous material associated with cellulose derivatives or compounded derivatives, 20 as a raw material. For instance, one available source of waste is the cuttings produced when making shoe stiffeners by impregnating or coating a fabric on one or both sides with a compounded cellulose derivative, such 25 as celluloid, and then cutting into the stiffeners. Such waste material may comprise a high grade cotton fiber which may be beaten and formed into a sheet having excellent characteristics. Another available source of 30 waste is the paper cuttings produced when making shoe stiffeners in accordance with the present invention.

The gelatinization of the cellulose derivative prior to the coating of the fibrous material may be accomplished by the use of suitable solvents for the derivative, whereupon 35 after coating of the fibrous material has been effected, the solvent may be vaporized, under elevated temperature conditions and while 40 effecting a recovery of the solvent, if desired. When loose, unwoven fiber in fluffy or bulk condition is employed as a raw material, sufficient solvent is preferably employed to produce a fairly thin solution, whereupon 45 fiber is added to the solution and uniformly distributed therethrough in order to effect a coating of substantially all the fibers with the cellulose derivative; and thereafter the 50 solvent is permitted to evaporate. The dried product is disintegrated into pieces of convenient size and is beaten in the presence of water to form a pulp capable of being formed into waterlaid sheets of uniform texture on a paper machine.

55 A specific example of procedure which gives a highly satisfactory product is carried out substantially as follows. One hundred parts of cellulose acetate is dissolved in sufficient "methyl-cellosolve" (a well known 60 solvent mixture) to produce a solution of a thin consistency. The acetate may be used in any suitable form, for example, in flaky, granular, or film form, and its solution may be effected by adding the solvent and permitting it to remain in contact with the acetate 70 under room temperature conditions for a sufficient period of time to ensure a complete solution. To the dissolved acetate is gradually added, with stirring, 100 parts of cellulosic fiber, such as cotton. For this purpose, a 75 mixing and kneading machine, such as a Werner and Pfleiderer, or dough-kneading machine, is preferably, though not necessarily employed. The viscosity of the solution is so increased by the addition of the fiber that when all the fiber has been incorporated therewith, a mass of spreadable consistency is obtained. The mass is then spread out by any suitable mechanical means, and permitted to dry, as a result of which is 80 found that setting into a hard, coherent sheet has taken place. The sheet is then cut into small pieces and added to a beater engine together with sufficient water to ensure circulation. The beater is initially operated for 85 about an hour with the roll raised sufficiently so that the pieces undergo a combing or teasing operation, which liberates the fibers carrying cellulose acetate attached thereto, in the form of a pulp. The beater roll is then 90 gradually lowered, so that at the end of about one hour it is in sufficiently close proximity with the bed-plate to effect a brushing of the fibers, whereupon beating is continued 95 until the stock is in a condition suitable for 100 forming into a sheet. The stock is then charged into the vat of a papermaking machine and run off into a waterlaid sheet of, say, about 50 points thickness. The sheet 105 is then dried and cut into stiffener blanks, which are preferably skived at their marginal portions. If desired, fabric such as cheesecloth may be adhesively secured to either or both faces of the sheet prior to cutting into blanks so as to avoid undue tackiness on the surface of the blanks after gelatinization of the cellulose derivative component by treatment with solvent. Box toe 110 blanks, packaged and sold in dry condition, 115 may be saturated with the solvent at the shoe factory immediately prior to pulling over or lasting; but it is generally preferable to treat the blanks with the solvent at the shoe stiffener factory, and then to package 120 the solvent-saturated stiffeners in hermetically sealed containers so that they will reach the shoe manufacturer in a limp condition ready for assembly with the shoe upper. When the treatment of the blanks is effected 125 at the point of use in the shoe factory, there may be insufficient time for the solvent to penetrate uniformly throughout the fibrous structure and accordingly incomplete gelatinization of the cellulose derivative component may occur. When, however, the solvent 130

treated blanks are supplied to the shoe manufacturer in closed containers and considerable time elapses after the treatment, the solvent vapors present in the closed containers ensure a complete and uniform gelatinization of the cellulose derivative component. The prolonged contact of the solvent with the cellulose fibers also appears to effect their softening. The blanks thus conditioned may accordingly be lasted with the shoe uppers more readily and satisfactorily.

The example hereinbefore given is merely illustrative, as it is possible to vary raw materials, proportions, and mode of treatment. Thus, the cellulose acetate employed as a raw material may be either chloroform-soluble or acetone-soluble, so that chloroform or acetone may be used in lieu of the methyl-cellosolve which is a solvent for both varieties of the acetate. Cellulose nitrate may be used instead of cellulose acetate, in which case methyl cellosolve or one of the usual nitrocellulose solvents may be employed; but cellulose acetate possesses the advantage over nitrocellulose, in that it is non-explosive and of comparatively low inflammability. Any suitable papermaking pulp may be used, including rag fibers, waste silk, and chemical wood pulps, such as kraft and sulphite pulp, but long-fibered stocks, such as cotton, manila, hemp, jute, ramie, are preferable, in that they afford a finished sheet of high tear resistance. Mixtures of long and short fibers may be used. Or the fiber may be in the form of a woven or knitted fabric or of a paper or felt, in which case such a base or foundation is impregnated or coated on one or both faces with the solution of cellulose derivative, and, after cutting into pieces of a size capable of being operated upon by the beater engine, is introduced into the engine and reduced to a pulp according to the desired beating schedule. The fiber surfaces of the foundation may be partially or completely coated with films of derivative after the treatment with the solution of derivative, but during the beating operation, fresh, uncoated fiber surfaces may be exposed, so that when the stock is in condition for forming into the sheet, it is composed of individual fibers or fiber aggregates, which are spotted with or carry discontinuous coatings of cellulose derivative.

I am aware of the fact that it has been proposed to incorporate cellulose derivatives, such as the nitrate and acetate, into felted fibrous foundations, as by dipping the prepared sheet material into a solution of such derivatives. Not only, however, is it difficult to effect a uniform impregnation of the sheet with a large amount of derivative by such a process, but a substantial proportion of the interstices or voids of the sheet are filled because the cellulose derivative exists as a continuous phase, so that subsequent

penetration by a solvent to effect gelatinization of the derivative is impeded. I am also aware of the fact that it has been proposed to incorporate cellulose derivatives, such as the nitrocellulose, in fibrous condition into paper stock in the beater engine prior to its sheeting in fibrous condition. Because the fibers of cellulose derivatives are weak or tender, however, the resulting sheet is quite fragile, especially when a substantial proportion of such fibers are used in the stock. Moreover, beating generates pulverized derivative, which, being unattached to the fibers of the stock, tends to flow out along with the water in which it is suspended during paper formation.

I claim:

1. Shoe stiffener material comprising a porous, waterlaid sheet of felted fibers to which is attached as a discontinuous phase a previously gelatinized cellulose derivative capable of again being gelatinized by a volatile solvent and of rendering said material stiff upon the evaporation of the solvent.

2. Shoe stiffener material comprising a porous, waterlaid sheet of felted cellulose fibers at least partially coated with a previously gelatinized cellulose derivative existing as a discontinuous phase and capable of again being gelatinized by a volatile solvent and of rendering said material stiff upon the evaporation of the solvent.

3. A box toe blank capable of being rendered limp by a cellulose acetate solvent and of setting in stiff condition, comprising a porous waterlaid sheet of felted cellulose fibers to which is attached as a discontinuous phase previously gelatinized cellulose acetate.

4. A box toe blank comprising a porous waterlaid sheet of fibers at least partially coated with a previously gelatinized cellulose derivative existing as a discontinuous phase and capable of again being gelatinized by a volatile solvent and of rendering said blank stiff upon the evaporation of the solvent, said derivative being present in amount by weight approximately equal to that of the weight of the fiber.

5. A process which comprises beating fibrous material coated with a previously gelatinized cellulose derivative capable of again being gelatinized by a volatile solvent, and sheeting the beaten stock on a paper machine.

6. A process which comprises gelatinizing a cellulose derivative with a volatile solvent, applying the gelatinized derivative to fibrous material, beating the fibrous material in the presence of water to form a pulp, and sheeting the pulp on a paper machine.

7. A process which comprises gelatinizing a cellulose derivative with a volatile solvent, mixing loose cellulose fiber with the gelatinized derivative, beating the mixture

in the presence of water to form a pulp, and sheeting the pulp on a paper machine.

8. A process which comprises treating a cellulose derivative with sufficient volatile solvent to form a thin solution, admixing cellulose fiber with the solution to produce a mass of spreadable consistency, evaporating the volatile solvent to effect a setting of the mass, beating the set product in water to form a pulp, and sheeting the pulp on a paper machine.

9. A process which comprises treating a paper-making fibrous material with a gelatinized cellulose derivative capable of again being gelatinized by a volatile solvent, beating the treated fiber in the presence of water to form a pulp, sheeting the pulp on a paper machine, and cutting the sheet into shoe stiffeners.

20 10. A process which comprises dissolving a cellulose derivative in a volatile solvent, coating a paper-making fibrous material substantially uniformly with the solution, evaporating the solvent, beating the material 25 in the presence of water to form a pulp, sheeting the pulp on a paper machine, cutting the sheet into shoe stiffeners, and treating the stiffeners with the volatile solvent to effect a gelatinization of the cellulose derivative.

In testimony whereof I have affixed my signature.

FRANK O. WOODRUFF.

35

40

45

50

55

60

65